

## UNITED STATES PATENT OFFICE

GEORGE A. RICHTER AND MILTON O. SCHUB, OF BERLIN, NEW HAMPSHIRE, ASSIGNEES  
TO BROWN COMPANY, OF BERLIN, NEW HAMPSHIRE, A CORPORATION OF MAINE

## PROCESS OF CHEMICALLY TREATING AND BLEACHING CELLULOSE PULP

No Drawing.

Application filed June 6, 1928. Serial No. 283,452.

This invention relates to the production of a bleached cellulose pulp of high cleanliness, whiteness, and low copper number.

In our Patent No. 1,639,704, dated August 23, 1927, it is disclosed that when free alkali is present during the bleaching of cellulose pulp, a product of high whiteness may be obtained without injury to the strength of the fibers and without lowering the alpha cellulose content of the pulp through the formation of oxycelluloses. The free alkali is preferably added to the bleach liquor at the start of bleaching and somewhat in excess of the amount necessary to be gradually consumed by reaction with acidic constituents initially present in the unbleached pulp or formed during bleaching, so that a distinctly alkaline condition is maintained throughout the bleaching operation. The alkali apparently makes the reaction between the bleach and pulp more selective in so far as the removal of impurities from the pulp is concerned. It also appears to have a solvent effect upon such oxycelluloses as may be present in the pulp at the start of bleaching, or as may be formed during bleaching. This patent further teaches the fact that higher temperature may be safely used during bleaching if free alkali be present in the bleach liquor, thereby eliminating the necessity for refrigerating the bleach liquor in hot weather, especially when stock is being bleached at a high density. Because of the protective influence which the alkali exercises over the cellulose, danger of local overbleaching is avoided, so that raw stock and strong bleach liquor may be uniformly admixed even in the summer when local overbleaching would ordinarily be certain to occur, particularly during initial mixing of the comparatively high temperature stock, resulting in a weakened stock and in a comparatively high bleach usage. A further advantage resulting from the use of free alkali during bleaching is the reduction in the number of resinous specks usually associated with the fibers, and accordingly the production of a cleaner pulp.

We have now found that if an alkali such as caustic soda is added to the raw stock before the bleach liquor, and is allowed to remain

in contact therewith at about room temperature for several hours, it has better opportunity thoroughly to penetrate the stock and to loosen resinous specks. This initial treatment with alkali, while advantageous when using any type of bleach, is of marked advantage when calcium base bleach, such as calcium hypochlorite, is subsequently employed, for when the alkali and calcium hypochlorite are added simultaneously to the raw pulp, there is a tendency for the bleach to react with the resins to form insoluble resinates and oxidation products which become fixed on the pulp, thereby interfering to an appreciable extent with the solution or dispersion of the resins, and the attainment of high whiteness. Even when sodium hypochlorite bleach is subsequently used, the initial treatment with an alkali such as caustic soda is advantageous, in that the resins are peptized and brought into a condition more susceptible to attack and removal by the bleach. The stock is preferably washed after the initial treatment with alkali, as resinous and other coloring substances are loosened thereby and may be readily removed. This not only permits subsequent bleaching to be done with less bleach than usual, but makes possible the production of an unusually white and clean pulp of high strength and low copper number.

The following are typical procedures such as have been studied in the laboratory and carried out in the mill on a large scale.

## Example I

A raw or unbleached sulphite pulp prepared from spruce chips as usual was treated as a suitably flowable aqueous pulp suspension, for instance at a stock density of 11%, at a temperature of 80° F. with 3/4% caustic soda (all chemical percentages are based on air-dry weight of the pulp used as a raw material). At the end of two hours, 1/2% caustic soda had been consumed. To the pulp was then added 15% calcium hypochlorite bleach and 1/2% caustic soda, and the mixture was allowed to react for eight hours at about 80° F. At the end of this period, it was found that 14% bleach and a total of 1% caustic soda

(including that previously added) had been consumed. The bleached stock was then washed, antichlored in sulphurous acid solution, and again washed. Although the 5 resin content of the original stock was 0.64% and was 0.5% after bleaching as usual in one step, the resin content of the product obtained by following the procedure herein outlined was 0.30%. The fact that the initial 10 treatment is effective in removing resins is clearly indicated by other observations. For instance, liquor expressed from a sample of pulp toward the end of the initial treatment was coffee-colored, and when evaporated gave 15 a dirty brown residue, rich in resin. Observation of the product obtained in the example cited under the microscope indicated that its speck count was materially lower than that of the raw stock as such, or even 20 after it had been bleached as usual in one step. The copper number of the raw stock when bleached as usual was 3.54, whereas that of the product obtained in the example 25 was 2.56.

25 *Example II*

A stock similar to that used in the foregoing example was initially treated with alkali as therein described, was then washed, 30 and treated for eight hours at a stock density of 11% and at a temperature of 80° F. with calcium hypochlorite bleach liquor containing 15% bleach and 1/2% caustic soda. Practically all of the bleach and caustic soda was 35 consumed. The bleached stock was then washed, antichlored, and again washed as in the foregoing example. It showed a material decrease in speck count and had a copper number approximately that of the product obtained in the foregoing example. The 40 reduction in the speck count is quite significant, for the specks eliminated in this treatment are of a resinous character, which are not removed by the rifflers in the mill which take out most of the other specks.

45 The strength and tear resistance of samples of the beaten product obtained in both examples were substantially similar to that of the product obtained by bleaching in the usual way, but the whiteness of the products obtained by processing according to the examples cited was markedly higher.

In a mill where a continuous process is being practised, about 3/4% caustic soda may be added to the raw sulphite stock entering 50 the system at 12% consistency and at about 70° F. At a point in the system reached by the pulp about two hours later, about 12% to 15% bleach may be added and the temperature raised to 80° F. About 1/2% of the caustic initially added will be consumed in the two-hour treatment before the bleach is added, but the stock will remain in a distinctly alkaline condition until practically all 55 the bleach is consumed.

60 In addition to the advantages hereinbe-

fore enumerated resulting from the application of the process of our invention, we have found that in actual mill practice we produce a final product of higher pH value than that associated with pulp bleached in the usual way. Thus, the raw stock bleached in the usual way resulted in a dry sheet of pulp, usually termed "drier sheet" in the trade, having a pH value of about 3.2 to 3.6 when tested by staining with bromo-cresol green, 70 but when processed as herein described, resulted in a dry sheet of pulp having a pH value of about 4.8 to 5.5. The higher pH value connotes greater stability in the pulp. Results obtained from large scale tests have shown that the stock of higher pH value will better endure a long continued beating. When beaten, for example, together with rag stock, as is done in mills of limited beater capacity, the wood pulp fibers still have good 80 strength when the tough rag fibers have been properly hydrated.

The process of the present invention has especial utility when applied in the treatment of raw sulphite pulp to produce a product which may be hydrated or gelatinized as readily as the usual sulphite pulp and which is suitable as for the manufacture of hard, ratty papers of good strength and tear resistance. Our product is, moreover, superior 90 in the important characteristics of whiteness and cleanliness. The initial treatment of the raw pulp with weak solutions of alkali at about room temperature, as herein described, does not change the character of the fiber as to its alpha cellulose or pentosan content to a pronounced degree, but is more especially effective in the removal, or in facilitating the subsequent removal by bleaching, of troublesome bleach-resisting and coloring impurities which otherwise require a more drastic bleaching treatment and cause a product of inferior whiteness, cleanliness, and copper number, to result. Our process is practical 100 in that it may be carried out with a low alkali and bleach consumption, without the use of heat, and without requiring equipment other than that usually employed in a bleaching process.

110 While in the specific examples given the alkalinity of the dilute solution at about room temperature used in the treatment of the pulp and in maintaining the bleach liquor alkaline is afforded by caustic soda, other chemicals, such as sodium carbonate, sodium phosphate, or borax may be used for this purpose. Again, while the specific examples deal with the use of sulphite pulp as a raw material, and a process comprising essentially only the chemical treatment of bleaching after the initial alkali treatment, other pulps may be used as a raw material and other chemical treatments may be advantageously included. For instance, the step of treating pulp with 120 a dilute caustic soda solution at about room 125 130

- temperature may be included in a pulp refining process which comprises the digestion of wood pulp at elevated temperature or at room temperature in an alkaline liquor of sufficient alkalinity or strength to refine the pulp to high alpha cellulose content, followed by the bleaching of the pulp, or in a pulp refining process which comprises the step of treating the raw pulp with bleach or chlorine water before the alkaline refining treatment. For instance, raw sulphite stock may be allowed to react with 1% caustic soda at a stock density of about 10% and at about 70° F. for about four hours, whereupon it may be washed to remove dark-colored, turbid reaction products. It may then be subjected to a series of refining treatments, including a treatment with chlorine, a washing treatment, alkaline digestion at high temperature, another washing treatment, a bleaching treatment, and a final washing treatment. If desired, the treatment with dilute alkali at room temperature may be performed after the chlorine treatment, or immediately before bleaching, rather than upon the raw stock. So, too, this treatment may be included in a refining process which involves the use of kraft pulp as a raw material and the bleaching of such pulp in a series of distinctly alkaline bleach liquors, the treatment being introduced before the series of bleaching is started or between the bleachings of the series. It may also be included as a preliminary step in a process which involves the bleaching of pulp in two steps, using chlorine water and hypochlorite bleach liquor in the order given, or vice versa, the bleach liquor preferably being maintained alkaline during the entire bleaching operation.
- Having thus described certain modes of practising this invention, it is evident to those skilled in the art that various changes and modifications might be made therein without departing from the spirit or scope of invention as defined in the appended claims.
- What we claim is:
1. A process which comprises treating unbleached sulphite pulp at about room temperature as a flowable aqueous pulp suspension in a solution containing not more than about  $\frac{1}{2}\%$  to 1% caustic soda based on the weight of air-dry pulp, washing the pulp, and bleaching the pulp.
  2. A process which comprises treating unbleached sulphite pulp at about room temperature as a flowable aqueous pulp suspension in a solution containing not more than about  $\frac{1}{2}\%$  to 1% caustic soda based on the weight of air-dry pulp, washing the pulp, and bleaching the pulp in a distinctly alkaline bleach liquor.
  3. A process which comprises treating unbleached sulphite pulp at about room temperature with a solution of caustic soda of such low alkalinity that practically no refinement of the pulp is effected but much of its resin content loosened, washing the pulp free of solution and loosened resinous matter, and bleaching the pulp.
  4. A process which comprises treating unbleached wood pulp at about room temperature with a solution of alkali of such low alkalinity that practically no refinement of the pulp is effected but much of its resin content loosened, and bleaching the pulp.
  5. A process which comprises treating unbleached wood pulp at about room temperature with a solution of alkali of such low alkalinity that practically no refinement of the pulp is effected but much of its resin content loosened, and bleaching the pulp in a calcium hypochlorite bleach liquor.
  6. A process which comprises treating unbleached wood pulp at about room temperature as a flowable aqueous pulp suspension in an alkaline solution whose alkali content does not exceed about 1% caustic soda equivalent based on the weight of dry pulp, thereby loosening impurities of the nature of resins from the pulp while substantially preserving its alpha cellulose content, and then bleaching the pulp.
  7. A process which comprises treating unbleached wood pulp at about room temperature as a flowable aqueous pulp suspension in an alkaline solution whose alkali content does not exceed about 1% caustic soda equivalent based on the weight of dry pulp, thereby loosening impurities of the nature of resins from the pulp while substantially preserving its alpha cellulose content, and then bleaching the pulp in a calcium hypochlorite bleach liquor.
- In testimony whereof we have affixed our signatures.
- GEORGE A. RICHTER.  
MILTON O. SCHUR.